

# United States Patent

[19]

Gribens et al.

[11] 3,888,380

[45] June 10, 1975

[54] POLYEPICHLOROHYDRIN AEROSOL  
GASKETS

[75] Inventors: **Joel A. Gribens**, Framingham;  
**Gregory P. Cogliano**, Canton, both  
of Mass.

[73] Assignee: **W. R. Grace & Co.**, Cambridge,  
Mass.

[22] Filed: **July 25, 1974**

[21] Appl. No.: **491,748**

## Related U.S. Application Data

[62] Division of Ser. No. 413,654, Nov. 7, 1973.

[52] U.S. Cl. .... **220/81 R; 222/402.1**

[51] Int. Cl. .... **B65d 7/34**

[58] Field of Search ..... **260/2 A; 264/268;**  
**220/81 R; 222/402.24, 402.1**

## References Cited

### UNITED STATES PATENTS

2,456,972 12/1948 Maeder et al. .... **264/268 X**

|           |        |                 |           |
|-----------|--------|-----------------|-----------|
| 3,024,949 | 3/1962 | Sagarin .....   | 222/394   |
| 3,135,705 | 6/1964 | Vandenberg..... | 260/2 A   |
| 3,145,011 | 8/1964 | Kappel.....     | 251/349   |
| 3,269,616 | 8/1966 | West .....      | 222/394   |
| 3,817,908 | 6/1974 | Guzy .....      | 260/37 EP |

## OTHER PUBLICATIONS

Maeda, "Characteristics of Various Synthetic Rubbers," Chem. Abstracts 68, 105861p (1968).

Primary Examiner—Morris Liebman

Assistant Examiner—E. A. Nielsen

Attorney, Agent, or Firm—Armand McMillan; C. E. Parker

## [57] ABSTRACT

Solutions of polyepichlorohydrin can be lined in the gasket channel of aerosol mounting cups by conventional lining equipment to yield gaskets with gas retention properties superior to those of neoprene gaskets.

1 Claim, No Drawings

**POLYEPICHLOROHYDRIN AEROSOL GASKETS**

This is a division of application Ser. No. 413,654, filed Nov. 7, 1973.

**THE PRIOR ART**

Pressurized aerosol containers are widely used to package and dispense an ever-increasing variety of materials. In these containers, the product to be dispensed is confined under pressure by means of a volatile propellant and is discharged in a controlled manner through a valve-actuated orifice.

A typical aerosol unit is composed of a hollow cylindrical container closed at one end and provided with an opening at its opposite end for receiving a dispensing valve assembly. A metal mounting cup serves as a closure for the container and also as a support for the valve assembly which is tightly fitted within an aperture centrally located in the cup. The mounting cup carries an annular gasket adapted at its outer edge to be crimped to the walls forming the opening in the container and thereby form a seal upon crimping.

The gasketing material used in aerosol mounting cups must be elastic and resilient. It must be capable of yielding under deforming forces to establish a satisfactory seal when the cup is crimped to the container. It must also be capable of maintaining the seal during normal storage periods. Often selected for this function are gaskets prepared from solvent-based rubber compositions which comprise an elastomer dissolved in a volatile organic solvent. The compositions may also contain pigments, fillers, curing agents and other conventional compounding ingredients. To prepare gaskets from an elastomeric composition, a band of the fluid composition is deposited in the annular channel of the mounting cup while the cup is being rotated beneath a metering nozzle through which the composition flows to form a continuous annular deposit. This deposit is subsequently converted into a dry solid elastomeric sealing mass by expulsion of the solvent and cure at elevated temperatures.

Because of superior resistance to oxidation and to oils and propellants as well as to various other chemicals commonly found in aerosol containers, neoprene (a chlorobutadiene polymer) has become the favored elastomer in this type of composition. Nevertheless, because of the great variety of materials and conditions encountered in aerosol packaging, the quest for improved gasketing materials continues.

**SUMMARY OF THE INVENTION**

It has now been discovered that polyepichlorohydrin compounds in solution form can be rapidly applied to the gasket channel of aerosol can valve mounting cups to yield, after drying and curing, gaskets with superior gas retention properties.

**DETAILED DESCRIPTION**

The compositions with which the benefits of the present invention can be obtained are solutions of polyepichlorohydrin elastomer in an organic liquid such as toluene. The polymer solutions are prepared typically in the following manner:

**POLYEPICHLOROHYDRIN COMPOUND**

The following chemicals, in the proportions listed, are milled on a Banbury mixer for five minutes with the temperature not exceeding 180°F:

| Ingredients                | Parts by Weight |
|----------------------------|-----------------|
| Polyepichlorohydrin rubber | 100.0           |
| Zinc stearate              | 1.0             |
| Magnesium oxide            | 5.0             |
| Carbon black               | 30.0            |
| 2-Mercaptimidazoline       | 1.5             |

10 The rubber compound thus obtained is then milled into a sheet, chopped and dissolved in toluene to yield a solution with a solids content of about 38 percent.

15 The rubber used for this compound is an amorphous epichlorohydrin homopolymer having a molecular weight of about 5,000 in the raw state. Suitable elastomers of that type differ from other conventional polyepichlorohydrins in that they are neither low molecular liquids nor hard crystalline materials. These usable elastomers are prepared, for example, in an inert 20 organic solvent at moderate temperatures (30° to 100°C) in the presence of a small quantity of an organoaluminum catalyst modified according to the method described in U.S. Pat. No. 3,135,705. The polymer may contain a minor quantity of units derived from ethylene oxide and the molecular weight may vary 25 within the range of about 4,000 to 20,000.

25 As to the rest of the ingredients formulated into the compound being described, they will be recognized as conventional rubber compounding materials in the nature of fillers, plasticizers, curing agents and the like. 30 As such, it is contemplated that they may be omitted and replaced by equivalent conventional substances without unduly affecting the utility of the composition.

**HIGH NEOPRENE COMPOUND**

35 A polychloroprene rubber content solution was prepared according to Example 3 of U.S. Pat. No. 3,748,297. The ingredients employed were the following:

| Ingredients                                 | Parts by Weight |
|---------------------------------------------|-----------------|
| Polychloroprene (Neoprene GN)               | 100             |
| Paraffin wax                                | 2.0             |
| Sodium acetate                              | 1.5             |
| Magnesium oxide                             | 8.0             |
| Tetraethylthiuram disulfide                 | 2.5             |
| Piperidinium-pentamethylene dithiocarbamate | 2.0             |
| Zinc oxide                                  | 5.0             |
| Diethyl phthalate                           | 7.4             |
| Silica gel                                  | 0.1             |
| Zinc resinate                               | 0.3             |
| Xylene                                      | 200             |
| 2-Mercaptobenzothiazole                     | 2.0             |
| Calcium carbonate                           | 50              |

55 These ingredients were mixed and dissolved in the conventional manner disclosed in U.S. Pat. No. 3,389,113, described below.

**LOW NEOPRENE COMPOUND**

60 A compound was prepared according to the method described in Example 1 of U.S. Pat. No. 3,389,113:

| Ingredients                   | Parts by Weight |
|-------------------------------|-----------------|
| Polychloroprene (Neoprene GN) | 100             |
| Sodium Acetate                | 1.5             |
| Paraffin wax                  | 2.0             |
| Buca clay                     | 99.8            |

-Continued

| Ingredients                                            | Parts by Weight                     |
|--------------------------------------------------------|-------------------------------------|
| Diethyl Phthalate (DOP)                                | 48.7                                |
| Light calcined magnesium oxide                         | 4.0                                 |
| Zinc Oxide                                             | 5.0                                 |
| Tetraethylthiuram disulfide (peptizer)                 | 2.5                                 |
| Piperidinium pentamethylene dithiocarbamate (peptizer) | 2.0                                 |
| Zinc resinate, 1.6% in DOP                             | 2.0                                 |
| Precipitated silicon dioxide                           | 0.1                                 |
| Toluene                                                | to about 57% total solids by weight |

The polymer, paraffin wax, sodium acetate and about 80 parts of the clay were milled together on a two-roll rubber mill. A blend containing the magnesium oxide and small portions of diethyl phthalate and zinc resinate solution were added to the rubber mix. After a smooth working sheet was obtained, the batch was transferred to an internal type mixer. Another blend containing the silicon dioxide, zinc oxide, a small portion of plasticizer and the remaining zinc resinate solution was then added along with the peptizers and the remaining clay and plasticizer. After mixing was complete, the batch was solvated in the toluene.

#### EXAMPLE 1

To test the rubber compounds just described and compare their performance as gaskets, the solutions were lined through a Dewey and Almy electropneumatic nozzle into the gasket channel of a number of aerosol mounting cups. The lined cups were then dried and cured according to the following standard laboratory schedule:

|        |   |         |
|--------|---|---------|
| 1 hour | — | air dry |
| 1 hour | — | 155°F   |
| 1 hour | — | 200°F   |
| 1 hour | — | 325°F   |

except that in the case of the polyepichlorohydrin compound, the last hour of treatment was at 347°F.

The resulting gaskets has the following dimensions and wet weight:

|                     | Thickness  | Wet film Weight |
|---------------------|------------|-----------------|
| Polyepichlorohydrin | 0.016 inch | 645 mg          |
| High neoprene       | 0.020      | 600 mg          |
| Low neoprene        | 0.025      | 500 mg          |

Aerosol cups lined with gaskets made from the three compounds of interest were crimped on aerosol cans in the conventional manner. The tightness of the crimp, although always necessarily greater in the case of the polyepichlorohydrin compound due to the thinner gasket yielded, was varied in terms of the crimp diameter and crimp depth within the following limits:

|                              | Crimping Condition |                 |
|------------------------------|--------------------|-----------------|
|                              | Depth (inch)       | Diameter (inch) |
| Polyepichlorohydrin (HYDRIN) | 0.180              | 1.070           |
|                              | 0.170              | 1.060           |
| Polychloroprene-high (PCHi)  | 0.210              | 1.070           |
| Polychloroprene-low (PCLo)   | 0.200              | 1.060           |

Each compound and each crimping condition was then tested against three different packs for leakage. The packs used were: (1) P12, difluorodichloromethane alone; (2) P12/EtOH, P12 and ethyl alcohol; and (3) P11/P12/MeCl, P12 with trichlorofluoromethane and methylene chloride.

The materials tested, the conditions and the results obtained are summarized in the next table. The results are stated in terms of average weight loss and number of can failures for each set of eight cans tested at the crimping and pack conditions indicated. The weight loss figures are given in milligrams of fluid lost during a period of 52 weeks of storage at 100°F. Failures are cans which either lost more than 5.5 g of fluid during that storage period or were seen bubbling within seven minutes of immersion in a 140°F bath.

TABLE I

| Compound | Depth (inch) | Diameter (inch) | Pack         | (Eight Cans Per Condition) |          |
|----------|--------------|-----------------|--------------|----------------------------|----------|
|          |              |                 |              | Average Wt. Loss (mg)      | No. Fail |
| PCHi     | 0.210        | 1.070           | P12/P11/MeCl | 2,768                      | 3        |
| HYDRIN   | 0.180        | 1.070           | P12/P11/MeCl | 518                        | 0        |
| PCLo     | 0.210        | 1.070           | P12/P11/MeCl | 3,426                      | 0        |
| PCHi     | 0.210        | 1.070           | P12/P11/MeCl | 3,389                      | 4        |
| HYDRIN   | 0.180        | 1.070           | P12/P11/MeCl | 621                        | 0        |
| PCLo     | 0.210        | 1.070           | P12/P11/MeCl | 2,918                      | 1        |
| PCHi     | 0.200        | 1.060           | P12/P11/MeCl | 653                        | 0        |
| HYDRIN   | 0.170        | 1.060           | P12/P11/MeCl | 980                        | 0        |
| PCLo     | 0.200        | 1.060           | P12/P11/MeCl | 2,740                      | 0        |
| PCHi     | 0.200        | 1.060           | P12/P11/MeCl | 851                        | 0        |
| HYDRIN   | 0.170        | 1.060           | P12/P11/MeCl | 704                        | 0        |
| PCLo     | 0.200        | 1.060           | P12/P11/MeCl | 3,202                      | 1        |
| PCHi     | 0.210        | 1.070           | P12/ETOH     | 2,182                      | 3        |
| HYDRIN   | 0.180        | 1.070           | P12/ETOH     | 26                         | 0        |
| PCLo     | 0.210        | 1.070           | P12/ETOH     | 3,468                      | 3        |
| PCHi     | 0.210        | 1.070           | P12/ETOH     | 1,128                      | 6        |
| HYDRIN   | 0.180        | 1.070           | P12/ETOH     | 56                         | 0        |
| PCLo     | 0.210        | 1.070           | P12/ETOH     | 13,270                     | 5        |
| PCHi     | 0.200        | 1.060           | P12/ETOH     | 175                        | 0        |
| HYDRIN   | 0.170        | 1.060           | P12/ETOH     | 40                         | 0        |
| PCLo     | 0.200        | 1.060           | P12/ETOH     | 6,143                      | 3        |
| PCHi     | 0.200        | 1.060           | P12/ETOH     | 307                        | 0        |
| HYDRIN   | 0.170        | 1.060           | P12/ETOH     | 56                         | 0        |
| PCLo     | 0.200        | 1.060           | P12/ETOH     | 38,570                     | 8        |
| PCHi     | 0.210        | 1.070           | P12          | 40,000                     | 8        |
| HYDRIN   | 0.180        | 1.070           | P12          | 148                        | 0        |
| PCLo     | 0.210        | 1.070           | P12          | 6,568                      | 3        |
| PCHi     | 0.210        | 1.070           | P12          | 30,758                     | 8        |
| HYDRIN   | 0.180        | 1.070           | P12          | 98                         | 0        |
| PCLo     | 0.210        | 1.070           | P12          | 6,352                      | 4        |
| PCHi     | 0.200        | 1.060           | P12          | 2,424                      | 3        |
| HYDRIN   | 0.170        | 1.060           | P12          | 47                         | 0        |
| PCLo     | 0.200        | 1.060           | P12          | 2,337                      | 0        |
| PCHi     | 0.200        | 1.060           | P12          | 1,818                      | 1        |
| HYDRIN   | 0.170        | 1.060           | P12          | 68                         | 0        |
| PCLo     | 0.200        | 1.060           | P12          | 4,695                      | 2        |

An examination of these results in terms of average weight loss and can failures demonstrate the great superiority of polyepichlorohydrin gaskets over those of neoprene under all crimping and pack conditions tested. The results may be summarized by averaging the figures for each compound:

| Compound                           | Overall Propellant Losses | Can Failures (per 96 cans) |
|------------------------------------|---------------------------|----------------------------|
| Polyepichlorohydrin                | 280 mg                    | 0                          |
| Polychloroprene-High Concentration | 7,204 mg                  | 36                         |
| Polychloroprene-Low Concentration  | 7,807 mg                  | 30                         |

## EXAMPLE 2

The effect of filler and plasticizer level on the gas retention performance of polyepichlorohydrin aerosol gaskets was determined by preparing the various compositions shown in Table II and lining them in the manner already described in Example 1.

age 52-week propellant loss in milligrams shown by the nine cans in that unit. The second figure, that after the comma, shows the number of cans that have failed, either by bubbling within seven minutes of immersion in a 140°F bath or by losing more than 5.5 g of propellant within one year storage at 100°F. Data obtained under

TABLE II

|                      | 1     | 2     | 3     | 4     | 5     | 6     |
|----------------------|-------|-------|-------|-------|-------|-------|
| Epichlorohydrin      | 100.0 | 100.0 | 100.0 | 100.0 | 100.0 | 100.0 |
| Zinc Stearate        | 1.0   | 1.0   | 1.0   | 1.0   | 1.0   | 1.0   |
| Magnesium Oxide      | 5.0   | 5.0   | 5.0   | 5.0   | 5.0   | 5.0   |
| Calcium Carbonate    | 50.0  | 50.0  | 100.0 | 200.0 | 50.0  | 50.0  |
| Diethyl Phthalate    | 0     | 0     | 0     | 0     | 15.0  | 30.0  |
| 2-Mercaptimidazoline | 1.5   | 1.5   | 1.5   | 1.5   | 1.5   | 1.5   |
| Azelaic Acid         | 0     | 2.0   | 2.0   | 2.0   | 2.0   | 2.0   |

Gaskets made from these compositions were then tested under the twelve crimp and pack conditions listed in Table III:

TABLE IV

| Test Condition       | PCLo     | COMPOUND |         |         |         |        |         |
|----------------------|----------|----------|---------|---------|---------|--------|---------|
|                      |          | No. 1    | No. 2   | No. 3   | No. 4   | No. 5  | No. 6   |
| I                    | 245, 0   | 114, 0   | 206, 0  | 242, 0  | 285, 0  | 315, 0 | 253, 0  |
| II                   | 4177, 3  | 4122, 3  | 548, 1  | 4119, 3 | 3510, 3 | 469, 1 | 24, 0   |
| III                  | 911, 1   | 505, 1   | 239, 2  | 1865, 2 | 407, 1  | 30, 0  | 486, 2  |
| IV                   | 387, 0   | 174, 0   | 340, 0  | 258, 0  | 256, 0  | 398, 0 | 367, 0  |
| V                    | 416, 1   | 4124, 3  | 423, 1  | 35, 0   | 975, 2  | 35, 0  | 480, 3  |
| VI                   | 1870, 2  | 64, 1    | 431, 2  | 713, 2  | 2336, 3 | 75, 0  | 1875, 2 |
| VII                  | 254, 0   | 485, 0   | 195, 0  | 156, 0  | 203, 0  | 204, 0 | 178, 0  |
| VIII                 | 74, 0    | 501, 1   | 369, 1  | 1020, 2 | 503, 1  | 500, 1 | 353, 1  |
| IX                   | 2083, 2  | 98, 0    | 93, 0   | 530, 1  | 120, 1  | 97, 0  | 82, 0   |
| X                    | 625, 0   | 202, 0   | 333, 0  | 228, 0  | 232, 0  | 308, 0 | 267, 0  |
| XI                   | 711, 1   | 86, 0    | 7297, 4 | 1773, 2 | 7686, 6 | 483, 1 | 504, 1  |
| XII                  | 25665, 9 | 908, 2   | 51, 2   | 606, 1  | 4202, 5 | 150, 0 | 428, 1  |
| Average Loss         | 2943     | 949      | 877     | 963     | 1727    | 256    | 442     |
| No. Fail/ Total Cans | 19/108   | 11/108   | 13/108  | 22/108  | 22/108  | 3/108  | 10/108  |

45

TABLE III

| Condition | Pack         | Depth (inch) | Diameter (inch) |
|-----------|--------------|--------------|-----------------|
| I         | P12/P11/MeCl | 0.200        | 1.070           |
| II        | P12/ETOH     | 0.200        | 1.070           |
| III       | P12          | 0.200        | 1.070           |
| IV        | P12/P11/MeCl | 0.200        | 1.060           |
| V         | P12/ETOH     | 0.200        | 1.060           |
| VI        | P12          | 0.200        | 1.060           |
| VII       | P12/P11/MeCl | 0.190        | 1.070           |
| VIII      | P12/ETOH     | 0.190        | 1.070           |
| IX        | P12          | 0.190        | 1.070           |
| X         | P12/P11/MeCl | 0.190        | 1.060           |
| XI        | P12/ETOH     | 0.190        | 1.060           |
| XII       | P12          | 0.190        | 1.060           |

The results of these tests in terms of average propellant weight loss and number of can failures for each compound under each condition are reported in Table IV. Nine cans were tested for each compound under each condition to give a total of 108 test cans per compound. The first figure in each result entry is the aver-

age 52-week propellant loss in milligrams shown by the nine cans in that unit. The second figure, that after the comma, shows the number of cans that have failed, either by bubbling within seven minutes of immersion in a 140°F bath or by losing more than 5.5 g of propellant within one year storage at 100°F. Data obtained under

identical conditions with gasket of polychloroprene-low concentration composition (PCLo) are included for comparison purposes.

Again, on comparison of the six polyepichlorohydrin compositions to polychloroprene, the performance of the gaskets of the invention as summarized by the average loss for all conditions and by the total of can failures is clearly demonstrated except in the case where an extremely high level of filler is used (compositions 4).

It also becomes apparent that variations in the nature and level of ingredients of the gasketing formula of the invention can be carried out by the man skilled in the art without departing from the scope of the invention as claimed.

What we claim is:

- An aerosol can valve-mounting cup equipped with an annular gasket which has been deposited into the annular channel of the cup in the form of a solution of an amorphous polyepichlorohydrin elastomer having a molecular weight within the range of about 4,000 to about 20,000, the solution having been subsequently dried and the dry elastomer cured in situ at elevated temperature.

\* \* \* \* \*